

## UNITED STATES PATENT OFFICE

JULIUS BEKK, OF BERLIN-STEGLITZ, GERMANY, ASSIGNOR TO THE FIRM DR. BEKK & KAULEN CHEMISCHE FABRIK G. M. B. H., OF BERLIN-LICHTERFELDE, GERMANY

PROCESS OF ETCHING PRINTING FORMS FOR INTAGLIO PRINTING, PLANOGRAPHIC PRINTING, AND THE LIKE

No Drawing. Application filed January 18, 1929, Serial No. 333,527, and in Germany January 24, 1928.

In manufacturing printing forms for intaglio printing, planographic printing and the like by mechanical or photochemical processes, the procedure, as is known, has in 5 many cases been to treat the forms covered with a developed copying layer with a suitable etching substance, e. g. with chloride of iron or nitric acid or the like. The application of such etching substances on forms 10 made of zinc, copper or the like is, however, connected with considerable difficulties, especially for this reason that the etching effect is easily carried too far, and that under such circumstances also such parts of the 15 plate or the like where etching is to be avoided may be affected.

I now have found that a perfectly satisfactory etching effect on such forms may be obtained if a mixture of chloride of iron and 20 nitric acid is used as the etching agent and preferably a highly concentrated chloride of iron solution in mixture with nitric acid. In this case the iron chloride may previously be dissolved in a small quantity of water or may 25 be mixed also in the solid state with the nitric acid. It is also possible to use, if desired, a special indifferent bearer for the etching agent in order to bring it in the form of a paste, salve or the like.

30 In the use of this etching agent the chloride of iron does not only assist in the etching of the printing plate or the like, but it also acts as a thickening means for the nitric acid and in this way prevents a too far going 35 effect of the nitric acid and an attacking of such parts of the plate which should not be etched, i. e. especially those that are yet covered with the copying layer. As has been proved, the same effect cannot be obtained 40 with the same security by the use of other thickening means.

To the etching agent a solution of iodine in iodide of potassium may be also added for the purpose of cleansing the metal and 45 of increasing its taking capacity for fat colours.

In practicing my invention it is essential that a highly concentrated solution of chloride of iron be used and that the nitric acid 50 should be present in the amount of 5% or

more. By a highly concentrated solution of chloride of iron I mean one containing at least 60% of the chloride. A preferred process is as follows:

75 parts of solid chloride of iron are dissolved in 25 parts of water, to which solution 10 parts of nitric acid of 1.4 spec. gravity are added. To this etching agent may further be added about 1 part of a solution of iodine in iodide of potassium. The etching means thus prepared may be made to act, according to requirements, up to several minutes on the printing form covered with a developed copying layer, e. g. a developed chrome-gelatine layer.

It is also within the meaning of the present invention to apply the process of etching according to the invention to such printing forms as are provided with a layer of a resinous substance or of varnish. The action of the etching agent on the plate or the like will in this case take place after the development of the plate covered with the resinous solution, and before the fatty colour is applied and before the treatment with alcohol.

Having now particularly described and ascertained the nature of my said invention, I declare that what I claim is:—

1. A process of etching metal printing forms for intaglio printing, planographic printing and the like, said printing forms being covered with a developed colloid layer on the exposed portions of the form, consisting in etching said metal forms with a mixture containing chloride of iron and nitric acid as the only essential ingredients.

2. A process of etching metal printing forms for intaglio printing, planographic printing and the like, said printing forms being covered with a developed colloid layer on the exposed portions of the form, consisting in etching said metal forms with a mixture of a solution containing at least 60% of iron chloride and at least 5% nitric acid.

3. A process of etching metal printing forms for intaglio printing, planographic printing and the like, said printing forms being covered with a developed colloid layer on the exposed portions of the form, which comprises etching said metal forms with a

mixture of chloride of iron, nitric acid and a solution of iodine in dissolved potassium iodide.

4. A process of etching metal printing forms for intaglio printing, planographic printing and the like, said printing forms being covered with a developed colloid layer on the exposed portions of the form, which comprises etching said metal forms with a mixture of a highly concentrated solution of iron chloride, nitric acid and a solution of iodine in dissolved potassium iodide.

In testimony whereof I have hereunto set my hand.

DR. JULIUS BEKK.

15

20

25

30

35

40

45

50

55

60

65